

March 24, 1959

G. B. HARES

2,879,420

IMAGE ORTHICON TARGET

Filed Aug. 28, 1957



INVENTOR.  
GEORGE B. HARES  
BY  
Clarence R. Petty, Jr.  
ATTORNEY

## 1

2,879,420

## IMAGE ORTHICON TARGET

George B. Hares, Corning, N.Y., assignor to Corning Glass Works, Corning, N.Y., a corporation of New York

Application August 28, 1957, Serial No. 680,745

2 Claims. (Cl. 313—68)

This invention relates to glass compositions and particularly to compositions of glasses suitable for the "target" in an image orthicon tube of improved design.

Such tubes are utilized in video cameras to convert an optical image into an electronic image for broadcasting purposes. Their general structure is well known to those skilled in the art pertaining to television and requires little amplification here. For a better understanding of the invention, however, reference is had to the accompanying drawing which is a schematic sectional view of an image orthicon tube showing its general structure.

In the drawing a glass tube or envelope generally designated 10 has a plane front end or face plate 11 having on its inner surface a photo-cathode 12 (shown in exaggerated thickness) consisting of a thin, continuous, semi-transparent layer usually comprising cesium, silver oxide and silver. Spaced from the photo-cathode is a glass target 13 (shown in exaggerated thickness) and improved composition for which forms the subject of this invention.

In a typical image orthicon tube, the target 13 is a circular membrane, which may be about 40 mm. in diameter and 3-5 microns thick, sealed to a supporting ring 14 of metal having a thermal expansion coefficient compatible with that of the glass. Such glass, heretofore used for the target, was normally composed of a soda-lime-silicate glass of the type used in making incandescent electric lamp bulbs, such as is described in Patent No. 1,369,988 and particularly in Example 4 of that patent.

In front of the target 13 and spaced about 50-100 microns therefrom is a very fine metal gauze 15 (shown in exaggerated thickness) having about 20 meshes per mm. with about 50-65% open area. In the opposite end of the tube 10, an electron gun 16 is provided with a grid 17 surrounding the aperture of the gun and a multi-stage electron multiplier 18.

In the operation of the image orthicon tube an optical image formed by a lens system (not shown) arranged in front of the face plate 11 is projected on the front surface of the photo-cathode 12. Photo-electrons thereby emitted from the rear surface of the photo-cathode strike the front face of the target 13 and cause the emission therefrom of secondary electrons in larger number than the photo-electrons. The emitted secondary electrons which are carried off by the metal gauze 15 leave electron deficiencies or positive charges on the front face of the target. Since the photo-electrons were compelled to pass through the metal gauze 15 on their way to the target 13, a pattern of individual positive charges thus remains on the front face of the target and delineates the image thereon.

Such charges are conducted perpendicularly but not laterally through the glass target to its rear face where they are neutralized by a scanning beam of low-velocity electrons provided by the electron gun 16. The electron

## 2

beam thus modulated is reflected to the grid 17 causing the emission of secondary electrons therefrom which are collected by the multiplier 18 and subsequently amplified for broadcasting.

5 Further details of the structure and operation of an image orthicon tube are described beginning at page 95 of R.C.A. Review, volume 10 (June 1949), in an article entitled "Development and Performance of Television Camera Tubes," by Janes, Johnson and Moore.

10 The proper functioning of the glass target depends upon the rapid transfer of the positive charges of the image perpendicularly through the thin glass membrane without substantial equalization or loss by transverse conductance. To prevent such transverse loss the glass should have a high volume resistivity. Too high a resistivity, however, can cause the incomplete discharge of the image by the scanning beam, a phenomenon known as "sticking." To facilitate the rapid removal of the image charge, the glass target is made as thin as possible. Suitable targets have a volume resistivity equal to about 11.4 to 12.1 for  $\log R$  at room temperature and a thickness of 3 to 5 microns.

15 The composition of glass suitable as a target is dependent upon its interaction with the photo-cathode during operation of the tube. The glass target must not contaminate the photo-cathode and thereby decrease its ability to emit photo-electrons. Also the glass must be of such a composition that reaction with the photo-cathode does not cause undesirable effects such as sticking of the image.

20 It has been found, that targets composed of the above-mentioned soda-lime-silicate glass tend to stick severely when used with improved photo-cathodes desirably containing a plurality of alkali metals. Likewise, it has been found that lithia-containing glass

25 targets are unsuitable because they poison the improved photo-cathode although they do not form sticking images. Such improved photo-cathodes have higher sensitivities than prior photo-cathodes but have not been successfully incorporated into an image orthicon tube because glass targets suitable therefor have heretofore been unavailable.

30 It is an object of the present invention to provide a glass composition suitable for a target in an image orthicon tube having a multi-alkali photo-cathode which will not form a sticking image nor poison the photo-cathode.

35 According to the invention such a glass consists essentially by weight of about 5%-65%  $\text{SiO}_2$ , about 25%  $\text{K}_2\text{O}$ , and about 10%-20%  $\text{TiO}_2$ .

40 While the stated proportion of  $\text{K}_2\text{O}$  is critical within a fraction of a percent for maintaining the proper coefficient of thermal expansion, the proportions of  $\text{SiO}_2$  may vary from 55% to 65% and of  $\text{TiO}_2$  from 10% to 20% without unfavorably affecting the thermal expansion coefficient and without unduly affecting the electrical resistivity and other physical properties.

45 Preferably, however, the glass consists essentially of about 60%  $\text{SiO}_2$ , about 25%  $\text{K}_2\text{O}$  and about 15%  $\text{TiO}_2$ .

50 Examples of glass compositions which can be used for targets to obtain the advantages of this invention can be prepared by melting the following batches:

|                                                            | 1    | 2    | 3     |
|------------------------------------------------------------|------|------|-------|
| Pulverized Sand.....                                       | lbs. | 275  | 597.7 |
| $\text{TiO}_2$ .....                                       |      | 100  | 149.4 |
| $\text{K}_2\text{CO}_3$ (57.3% $\text{K}_2\text{O}$ )..... |      | 196  | 399.8 |
| $\text{KNO}_3$ .....                                       |      | 33.6 | 42.6  |
| $\text{Sb}_2\text{O}_3$ .....                              |      | 2.5  | 5.0   |
|                                                            |      |      | 2.5   |

The glasses corresponding to the above batches, calcu-

lated in weight percent on the oxide basis, are as follows:

|                                | 1    | 2    | 3    |
|--------------------------------|------|------|------|
| SiO <sub>2</sub>               | 54.7 | 59.8 | 64.7 |
| K <sub>2</sub> O               | 24.9 | 24.9 | 24.9 |
| TiO <sub>2</sub>               | 19.9 | 14.8 | 9.9  |
| Sb <sub>2</sub> O <sub>3</sub> | 0.5  | 0.5  | 0.5  |

The Sb<sub>2</sub>O<sub>3</sub> functions only as a fining agent and has no substantial effect on the fundamental properties of the glass. The batches melt readily either in a closed pot or in a tank, preferably under oxidizing conditions, at about 1300°-1400° C. Preferably the glass should be stirred during melting and fining in order to minimize cords. The more important physical and electrical properties of the above glasses are as follows:

|                                                 | 1    | 2    | 3    |
|-------------------------------------------------|------|------|------|
| Softening point, °C.                            | 750  | 770  | 760  |
| Annealing point, °C.                            | 605  | 605  | 575  |
| Strain point, °C.                               | 575  | 570  | 540  |
| Expansion coeff. = $10^7$ ° C.                  | 102  | 100  | 101  |
| Resistivity, Log R <sub>25</sub> ° C. Ohm Cm.   | 12.1 | 11.8 | 12.1 |
| Resistivity, Log R <sub>250</sub> ° C. Ohm Cm.  | 6.7  | 6.5  | 6.7  |
| Resistivity, Log R <sub>1000</sub> ° C. Ohm Cm. | 5.5  | 5.3  | 5.5  |

What is claimed is:

1. In an image orthicon tube comprising a glass envelope containing in longitudinal arrangement a photocathode, a grid of fine metal gauze, a thin glass target and an electron gun, the improvement which comprises making said target of a glass consisting essentially by weight of 55%-65% SiO<sub>2</sub>, about 25% K<sub>2</sub>O and 10%-20% TiO<sub>2</sub>.
- 10 2. In an image orthicon tube comprising a glass envelope containing in longitudinal arrangement a photocathode, a grid of fine metal gauze, a thin glass target and an electron gun, the improvement which comprises making said target of a glass consisting essentially by weight of about 60% SiO<sub>2</sub>, about 25% K<sub>2</sub>O and about 15% TiO<sub>2</sub>.

References Cited in the file of this patent

UNITED STATES PATENTS

|    |           |           |       |               |
|----|-----------|-----------|-------|---------------|
| 20 | 2,617,058 | De Boer   | ----- | Nov. 4, 1952  |
|    | 2,617,954 | Rose      | ----- | Nov. 11, 1952 |
|    | 2,676,109 | Barnes    | ----- | Apr. 20, 1954 |
|    | 2,688,559 | Armistead | ----- | Sept. 7, 1954 |

UNITED STATES PATENT OFFICE  
CERTIFICATE OF CORRECTION

Patent No. 2,879,420

March 24, 1959

George B. Hares

It is hereby certified that error appears in the printed specification of the above numbered patent requiring correction and that the said Letters Patent should read as corrected below.

Column 2, line 47, for "5%-65%" read -- 55%-65% --; column 3, second table, first column thereof, fourth line, after "Expansion coeff." for " $\leq$ " read -- x --.

Signed and sealed this 9th day of June 1959.

(SEAL)  
Attest:

KARL H. AXLINE  
Attesting Officer

ROBERT C. WATSON  
Commissioner of Patents